

# UNITED STATES PATENT OFFICE.

LEON LILIENFELD, OF VIENNA, AUSTRIA-HUNGARY.

## ARTIFICIAL LEATHER AND COMPOSITION USED IN THE MANUFACTURE THEREOF.

1,217,123.

Specification of Letters Patent.

Patented Feb. 20, 1917.

No Drawing.

Application filed December 11, 1912. Serial No. 736,222.

*To all whom it may concern:*

Be it known that I, Dr. LEON LILIENFELD, a subject of the Emperor of Austria-Hungary, residing at No. 1 Zeltgasse, Vienna,

5 VIII, Austria-Hungary, have invented certain new and useful Improvements in Artificial Leather and Composition Used in the Manufacture Thereof, of which the following is a specification.

10 Oils and fats and their derivatives and more especially castor oil, have chiefly been used as agents for imparting softness and elasticity in the manufacture of artificial leather from colloided cellulose ester masses.

15 The use of those agents has the following disadvantages:—

Oils and fats and more especially castor oil, impart to the imitation leather an unpleasant smell which increases with the

20 lapse of time according as the oils and fats, and more especially castor oil, become rancid. Artificial leather made from colloided cellulose ester masses with the help of oils and fats, and more especially castor oil, is

25 of limited durability. In time the covering layers of such artificial leather usually become stiff, brittle and friable. The resistance of such leather to heat is also small; the leather becoming stiff and brittle after even

30 a short time.

The softening action of oils and fats, and more especially castor oil, and their derivatives is limited. The use of a larger quantity of such agents has the effect of dimin-

35 ishing the adhesion of the composition to its foundation. In other words, the layers peel off. Since oils and fats have no solvent action upon nitro-cellulose or celluloid the manufacture of such artificial leather re-

40 quires considerable quantities of volatile and expensive solvents.

The applicant has now discovered that by using phenol esters, and in particular those which remain liquid at 0° Centigrade,

45 wholly or partially instead of oils and fats, and more especially castor oil, all the above stated drawbacks are remedied and new advantages are obtained.

Above all, the softening action of these phenol esters is much greater than that of oils and fats and more especially castor oil, so that artificial leather made by the use of

a composition of matter containing a colloided cellulose ester mass and one or more phenol esters remaining liquid at a temperature of 0° C. is softer, more pliable and more resistant to scratching and rubbing than the artificial leather made by the use of the known masses. Now artificial leather made with the help of a composition of matter according to the present invention and containing a colloided cellulose ester mass and said phenol esters is perfectly free from smell, does not become stiff or brittle in storage, and can withstand perfectly temperatures of 100 degrees C. without becoming stiff or brittle.

A further advantage is that the said phenol esters have a solvent action upon nitro-cellulose and thus allow of effecting a saving in the quantities of volatile solvents used.

Another important advantage is that layers consisting of nitro-cellulose or celluloid and the said phenol esters have a good adhesion to viscose, and especially to viscose mixed with products described in the specification of Patent No. 1037158—for example the condensation products of Chinese wood oil with amino aromatic hydrocarbon derivatives, or hydroxyl derivatives of these, or rubber, gutta percha, balata, resins and similar materials; and further that layers of viscose mixed with said products adhere likewise very well to layers consisting of nitro-cellulose or celluloid and the said phenol esters.

Artificial leather and imitation wax cloth composed of layers composed of colloided cellulose ester mass, for example, nitrocellulose colloided with camphor or other colloiding agent and phenol esters which remain liquid at 0° C.; alternating with layers consisting of mixtures of viscose and products obtained by heating aromatic amines with Chinese wood oil and a condensing agent, are products valuable in the art, and are distinguished by their very great softness, pliability and gloss, and also cheapness.

In carrying out the manufacture of the new composition, a colloided cellulose ester mass such as nitro-cellulose or in general any cellulose ester colloided with camphor or other colloiding agent is dissolved in a suitable solvent, and to the solution there is

added a phenol ester which remains liquid at 0° C. Ortho-tricresyl-phosphate has been found especially suitable for this purpose. This solution, may be also mixed with other suitable binding agents (for instance, acetyl-cellulose, formyl-cellulose, caoutchouc, gutta-percha, drying oils and the like) or with filling substances for giving bulk (for instance, ground leather, powdered cork, asbestos, precipitated chalk, china-clay, etc.,) or with 5 pigments or coloring matters or with other softening agents (such as oils, fats, especially castor oil, glycérin, sugar, soaps and the like). The composition of matter thus obtained is applied to suitable foundation materials such as textile fabrics, paper, cotton or paper fleece, or the like, by hand or by means of suitable machinery, or it may be rolled thereon. The application of the 10 composition may be effected in one or more coats or layers. If the composition is applied in several layers the percentage either of nitro-cellulose or celluloid or of phenol esters which remain liquid at 0° C. or of 15 both may vary in any of the several layers.

Since the colloided cellulose ester mass, for example, nitrocellulose colloided with camphor or other colloiding agent when only mixed with the said phenol esters and well kneaded yield compositions or pastes capable of being applied or rolled on, there is no need to use volatile solvents, or if such are used the quantity employed may be very small.

35 The following are examples of the new composition of matter and the same are used in the manufacture of artificial leather:

#### Composition No. 1.

40 60 parts by weight of alcohol,  
30 " " " acetone,  
10 " " " powdered celluloid,  
10 " " " ortho-tricresylphosphate.

#### 45 Composition No. 2.

60 parts by weight of alcohol,  
30 " " " acetone,  
10 " " " powdered celluloid,  
50 5 " " " ortho-tricresylphosphate.

#### Composition No. 3.

55 40 parts by weight of glacial acetic acid,  
60 " " " alcohol,  
12 " " " powdered celluloid,  
12 " " " ortho-tricresylphosphate.

#### 60 Composition No. 4.

60 parts by weight of alcohol,  
30 " " " acetone,  
10 " " " powdered celluloid,  
65 10 " " " creosote phosphate.

#### Composition No. 5.

60 parts by weight of alcohol,  
30 " " " acetone,  
10 " " " powdered celluloid,  
10 " " " creosote carbonate. 70

#### Composition No. 6.

60 parts by weight of alcohol,  
30 " " " acetone,  
10 " " " powdered celluloid, 75  
10 " " " creosote oleate.

#### Composition No. 7.

1000 parts by weight of a substance produced by heating 100 parts by weight of Chinese wood oil with 200 parts by weight of ortho-toluidin and 11 parts by weight of zinc chlorid, washing in water and drying, are, while being stirred and kneaded together, heated to water bath temperature, 85 and then 550 parts by weight of soda-Turkey-red-oil of about 40 to 55 per cent. of dry residue and 6 to 10 per cent. of ash are added in several doses. Then 60 parts by weight 90 of a soda solution of 50° Bé. are added in several doses, and finally the mass is diluted by kneading with 800 parts by weight of water. The finished solution or emulsion may then be strained for the purpose of freeing it from impurities. 95

#### Composition No. 8.

100 parts by weight of Composition No. 7 are well mixed with 40 to 50 parts by weight 100 of a raw viscose containing 13 per cent. of cellulose.

#### Composition No. 9.

100 parts by weight of Composition No. 7 are well mixed with 75 to 100 parts by weight 105 of a raw viscose containing 13 per cent. of cellulose.

#### Artificial leather No. 1.

Composition No. 1 is mixed with a pigment for example soot, or with a pigment lake or the like and applied in one or more layers to a suitable textile fabric. If several layers are applied, each layer may be satined or calendered before applying the next layer. The pigment may also be previously ground with the ortho-tricresylphosphate. 110

#### Artificial leather No. 2.

1st layer, (bottom preparation) :—Composition No. 1.

2nd layer, (consisting of one to six coats) :—Composition No. 1 with the addition of a pigment or coloring matter.

3rd layer, (varnish layer) :—Composition 12 No. 2.

#### Artificial leather No. 3.

Composition No. 4 is mixed with a pigment (for instance soot or with a lake or the 13

like) and applied in one or more coats upon a suitable textile fabric.

*Artificial leather No. 4.*

5 Composition No. 5 is mixed with a pigment (for instance with soot or with a lake or the like) and applied in one or more layers upon a suitable textile fabric.

*Artificial leather No. 5.*

10 Composition No. 6 is mixed with a pigment (for instance with soot or with a lake or the like) and applied in one or more layers upon a suitable textile fabric.

15 The artificial leathers obtained may be calendered or pressed at the finish or between the several layers and finally marked with any desired leather graining or other design.

20 The superior durability of the products obtained by the use of the new composition for the manufacture of artificial leather and the like over those of existing processes is shown, for instance, by the following tests:

25 Artificial leathers made with the use of the new composition were heated together with samples of artificial leather which had been made exactly in the same manner but with the difference that pure castor oil was used instead of phenol esters. The samples of imitation leather were then heated with access of air to 100-105 degrees C. with the following result:

30 Whereas artificial leathers made with the new composition after fourteen days (at the end of which period the test was discontinued) showed no alteration whatever, appearance, softness, feel and fastness to rubbing remaining completely unchanged, the other similar leathers made with castor oil became hard and brittle after a period of only 17½ hours. After 29 hours these leathers broke when pulled, and after 53 hours the layer crumbled away altogether when rubbed.

45 What I claim is:—

1. A permanently soft and flexible composition of matter, viscous at ordinary temperature, containing nitrocellulose, a colloidal agent therefor and a phenol ester.

2. A permanently soft and flexible composition of matter, viscous at ordinary temperature, containing nitrocellulose, a colloidal agent therefor and a plurality of phenol esters.

3. A composition of matter for the manufacture of artificial leather and the like, containing a colloided cellulose ester mass and a phenol ester which remains liquid at a temperature of 0° C. in admixture with a solvent common to both, substantially as described.

4. A composition of matter for the manufacture of artificial leather and the like, containing a colloided cellulose ester mass,

and a plurality of phenol esters which remain liquid at a temperature of 0° C. in admixture with a solvent common to both, substantially as described.

5. A composition of matter, viscous at ordinary temperature, permanently soft and flexible, containing 100 parts of nitrocellulose, a colloidal agent therefor, and from 50 to 200 parts of a phenol ester.

6. A composition of matter viscous at ordinary temperature, permanently soft and flexible, containing 100 parts of nitrocellulose, a colloidal agent therefor, and from 50 to 200 parts of orthotrichresyl phosphate.

7. A composition of matter for the manufacture of artificial leather and the like, containing one hundred parts of nitrocellulose and from fifty to two hundred parts of a phenol ester which remains liquid at a temperature of 0° C. in admixture with a solvent common to both, substantially as described.

8. A composition of matter for the manufacture of artificial leather and the like, containing 100 parts of nitrocellulose and from 50 to 200 parts of orthotrichresyl phosphate in admixture with a solvent common to both, substantially as described.

9. A composition of matter for the manufacture of artificial leather and the like, containing a colloided cellulose ester mass and a phenol ester which remains liquid at a temperature of 0° C. and which acts as a softening agent, in admixture with further softening agents, binding agents, substances for giving bulk and coloring matters, substantially as described.

10. A composition of matter for the manufacture of artificial leather and the like, containing a colloided cellulose ester mass and a phenol ester which remains liquid at a temperature of 0° C. and which acts as a softening agent, in admixture with further softening agents, binding agents, substances for giving bulk, coloring matters and suitable solvents, substantially as described.

11. A product containing a flexible base, carrying thereupon, successive layers of plastic material, at least one of said layers comprising a colloided cellulose ester mass, and a phenol ester, liquid at 0° C.

12. A product comprising a fabric base, carrying thereupon, successive layers of plastic material, at least one of said layers comprising nitrocellulose, a colloidal agent therefor and trichresyl phosphate.

13. As a new product, artificial leather comprising a fabric coated with a mixture comprising a colloided cellulose ester mass and a phenol ester which remains liquid at 0° C.

14. As a new product of manufacture, artificial leather comprising a fabric coated with a mixture comprising a colloided cellu-

lose ester mass and a plurality of phenol esters which remain liquid at 0° C.

15. An artificial leather comprising a flexible base, and a permanently plastic composition coated thereupon, said composition comprising celluloid and a phenol ester which is non-volatile in storage at atmospheric temperature, which composition is stable and free from castor oil and similar

materials, and which artificial leather exhibits at least as great a resistance to scratching and rubbing as does real leather.

In testimony whereof I affix my signature in presence of two witnesses.

DR. LEON LILIENFELD.

Witnesses:

HERMAN WUNDERLICH,  
HANS JYRIKA.